

## UNITED STATES PATENT OFFICE

MARCEL VARINOIS, OF PARIS, FRANCE, ASSIGNOR TO SOCIÉTÉ ANONYME DES LABORATOIRES ROBERT & CARRIERE, OF PARIS, FRANCE

## STRING FROM ANIMAL ORIGIN AND PROCESS FOR MANUFACTURING THE SAME

No Drawing. Application filed July 5, 1929, Serial No. 376,294, and in France May 16, 1929.

The object of this invention is to provide a process for manufacturing strings and other flexible ties from material of animal origin.

5 This process, which is a result of investigations which I have made, aims especially at manufacturing strings intended to replace, on the one hand, those at present used in surgery under the name of "catgut", and, 10 on the other hand, those used in industry, especially for racket stringing and as harmonic strings with musical instruments.

Persons skilled in the art are aware that the latter, as hitherto manufactured, are constituted by suitably treated sheep guts. Such strings offer a plurality of deficiencies of which the principal ones are as follows:

They lack homogeneousness. In order to make them, sheep guts, or more precisely 20 the small intestine of sheep, are split lengthwise, an operation which frequently causes breaks so that, since every effort is made to use most advantageously thongs so obtained, catguts—as well as racket strings and harmonic strings—are in practice, constituted by pieces of guts of very unequal lengths. The finished product offers, therefore, a 25 number of breaks in continuity, and since a catgut is generally composed of 5 or 6 thongs twisted together, it will be readily realized that every break of continuity decreases the strength thereof by 1/5th or 1/6th, and often by far more whenever two 30 breaches of continuity happen to be somewhat proximate to one another.

With small gauge catguts obtained by twisting 2 or 3 thongs together strength may vary by 50% between one product and another.

40 In the second place, the finished products show inequalities as to gauge; in fact the sheep guts used come from animals differing as to age and size and are themselves of widely different dimensions. When such 45 guts are split, the thongs obtained are of very variable width since, on the one hand, the operation is mostly hand effected, and, on the other hand, the elasticity and strength of guts vary considerably from one sample 50 to another. By twisting such thongs to-

gether, strings are obtained some parts of which are of larger diameter than other parts, due to the fact that several thongs particularly wide or thick are assembled at one point, while other portions are far finer and, therefore, weaker.

In the third place, and on account of reasons resulting from the above recited facts, small pieces of guts simply cannot be used at all.

Lastly, as concerns surgical utilizations of such strings, that is to say of strings more especially known in practice as "catguts", sheep guts yield products which are very difficult, if not quite impossible, to be rendered thoroughly aseptic. As a matter of fact, sheep guts contain fecal matters which constitute a huge microbial colony since bacteria represent about 1/4th of the total volume of such matters; as soon as the animal 70 has been slaughtered many of said bacteria penetrate into the intestinal wall thereby enhancing decomposition of the carrión.

In order to rid the guts of their outer muscular tunic and of their inner mucous tunic, manufacturers leave them to cure for 48 hours in cold water; obviously this period of time allows bacteria to develop within tissues and incipient decomposition is what permits the outer and inner tunics to 80 be stripped from their backing. Lastly, all handlings are effected in water that could hardly completely remove fecal matters and bacteria unless absolutely prohibitive quantities of washing water were used.

85 The process which is the object of my invention consists in making use, for manufacturing surgical catguts, racket strings, harmonic strings, etc., of animal fibers, such as muscle fibers, fibers of various membranes, 90 intestinal fibers, and, especially, tendinous fibers.

As an example, I will hereinafter describe the chief operations involved in performing my process when animal tendons or 95 sinews are used as raw material.

I take said sinews as fresh as possible, rid them of all flesh and fat adhering thereto, next sterilize them and then put them to dry at a low temperature.

Once the sinews are dry, I laminate or card them in order to promote fiber dissociation, and when said separation has been completed by means of a fiber separator similar to those now in use for separating the fibers, vegetable textiles, very fine fibers are obtained, which may be, for instance, less than 1/10th of a millimeter in diameter.

Lastly, the fibers so obtained are twisted by the methods used in twine manufacturing so as to achieve strings of various sizes according to the purpose for which intended.

The above described process is also applicable to any fibers besides tendons or sinews; it will permit of making strings of regular and even thickness, homogeneous in character, very strong and of a length theoretically unlimited or, at any rate, independent from the constituent fiber lengths. Lastly, from the surgical point of view, such strings will be far more aseptic than cat-guts made of sheep guts.

Having now particularly ascertained and described the nature of my said invention as well as the manner in which the same is to be performed, I declare that what I claim is:

Claims.

1. A process for manufacturing strings, consisting in using fresh animal sinews, ridding them of all flesh and fat adhering thereto, and successively sterilizing them, drying them at a low temperature, separating the fibers and twisting the fibers to the desired size.

2. Strings for rackets, musical string instruments and for surgical purposes, made from fresh animal tendons or sinews whose fibers are cleaned, sterilized, dried at low temperature, separated and twisted to the desired size.

In testimony whereof I affix my signature.  
MARCEL VARINOIS.